

## UNITED STATES PATENT OFFICE

2,127,245

## ALLOY

Walter R. Breeler, Troy, N. Y., assignor to Lud-lum Steel Co., Watervliet, N. Y., a corporation of New Jersey

No Drawing. Application July 19, 1935,  
Serial No. 32,237

6 Claims. (Cl. 75—124)

My invention relates to alloy steels and particularly to steels having high resistance to hot oxidation, scaling, and corrosive loss by the attack of compounds containing lead at high temperatures. The alloy is particularly adapted for use in lead pots, pyrometer tubes and the like, and for exhaust valves, seat inserts and other parts of internal combustion engines which are subjected to contact with hot exhaust gases resulting from the combustion of gasoline containing lead anti-knock compounds. The alloys at present employed for these purposes are rather high priced, and one of the objects of my invention is to produce a relatively cheap material characterized by its resistance to hot oxidation and to hot lead compounds.

The essential ingredients of my alloy and the limits between which they are employed are as follows:

|     | Percent |      |     |     |    | Loss in weight (mg./sq.cm./min.) |                       |       |                         |    |
|-----|---------|------|-----|-----|----|----------------------------------|-----------------------|-------|-------------------------|----|
|     | C       | Si   | Cr  | Al  | Mn | Rock-well C                      | PbO·PbBr <sub>3</sub> | PbO   | 3PbO·2PbSO <sub>4</sub> |    |
| 0.3 | 2.8     | 20.4 | 3.1 | 8.9 | 25 | 1350°                            | 1580°                 | 1800° | 1800°                   | 10 |
| 0.9 | 0.6     | 20.8 | 3.1 | 9.6 | 21 | Nil                              | Nil                   | Nil   | 14.8                    | 15 |

as will be apparent from the following comparative tests of two alloys both of which contain chromium and manganese in about the same amounts but in one of which the aluminum content is 3.1% with a silicon content of 0.6%, and in the other alloy no aluminum is present, but the silicon content is 2.8%.

|     | C   | Si   | Cr  | Al  | Mn | Rock-well C | PbO·PbBr <sub>3</sub> | PbO   | 3PbO·2PbSO <sub>4</sub> |
|-----|-----|------|-----|-----|----|-------------|-----------------------|-------|-------------------------|
| 0.3 | 2.8 | 20.4 | 3.1 | 8.9 | 25 | 1350°       | 1580°                 | 1800° | 1800°                   |
| 0.9 | 0.6 | 20.8 | 3.1 | 9.6 | 21 | Nil         | Nil                   | Nil   | 14.8                    |

Neither of these alloys shows any loss in weight when subjected to lead oxy bromide at 1350° F. At 1580° F. the alloy without the aluminum shows a rather substantial loss while the other shows none. At 1800° F. the alloy without the aluminum but with fairly high silicon when subjected to lead oxide shows a loss exceeding three times that of the other, and at the same temperature with a mixture of lead oxide and lead sulphate the loss of the composition without the aluminum is about seventy times greater than the other.

In the preferred analysis range mentioned, and in the lower ranges of aluminum, chromium and manganese (especially aluminum), the alloy is readily forgeable and rollable. In the higher ranges of alloy content (especially aluminum) the alloy is more difficult to hot work and requires more care at this operation. However, in cases where hot working is impractical, the alloy may be readily cast and used in this form.

My alloy can be made by any of the well known methods of melting. For example, when using an electric arc furnace the aluminum may be added as metallic aluminum or aluminum alloy in the furnace itself, or the aluminum or an aluminum alloy may be added in the ladle. These additions are preferably made under protective slag coatings of such a nature that they will not react detrimentally with the aluminum steel and they should be of such composition as to dissolve or flux any undesirable oxides such as Al<sub>2</sub>O<sub>3</sub>. Instead of the electric arc furnace, induction furnaces may be used. Such equipment may or may not be used with controlled atmospheres.

What I claim is:

1. A readily forgeable alloy steel containing a

A preferred range of the above alloying elements is as follows:

|    | Percent |      |      |  |  |
|----|---------|------|------|--|--|
| 30 | C       | 2    | 1.0  |  |  |
|    | Mn      | 8.0  | 12.0 |  |  |
|    | Cr      | 18.0 | 22.0 |  |  |
|    | Al      | 1.5  | 3.5  |  |  |

While the foregoing are the only elements necessary to attain the objects of my invention, other elements, in quantities which do not appreciably affect the basic characteristics of the alloy, namely, resistance to hot oxidation and to lead compounds at high temperatures, may be incorporated if desired. Such elements as selenium, tellurium, phosphorus and sulphur, in quantities up to 0.30% will improve the machineability of the alloy, and nitrogen in quantities up to 0.3% will increase the strength at heat and also the hardness.

Silicon, of course, is always present in steels and irons, and while I prefer to keep the silicon under about 1%, the quantity in any case should be less than the aluminum content. I find that silicon in excess of the aluminum very greatly reduces the resistance of the alloy to corrosive loss when subjected to attack by lead containing compounds at high temperature. Silicon and aluminum are not interchangeable in the alloy

plurality of elements and characterized by its resistance to hot oxidation and corrosive loss when subjected to attack by lead containing compounds at temperatures of the order of the operating temperatures of exhaust valves in internal combustion engines; the only essential elements necessary to obtain such characteristics being carbon from 0.2% to 1%, manganese from 8% to 12%, chromium from 18% to 22%, aluminum from 1.5% to 3.5% with the balance substantially all iron; the aluminum content being in excess of the silicon content, if any, in said steel.

2. An internal combustion engine valve characterized by its high resistance to hot oxidation and corrosive loss when subjected to attack by lead containing compounds at temperatures of the order of the operating temperatures of exhaust valves in internal combustion engines; said valve comprising an alloy steel containing a plurality of elements of which the only essential elements necessary to obtain the foregoing characteristics are carbon from 0.05% to 3%, manganese from 2% to 20%, chromium from more than 5% to 35% and aluminum from 0.5% to 15%, with the balance substantially all iron; the aluminum content being in excess of the silicon content, if any, in said steel.

3. An internal combustion engine valve characterized by its high resistance to hot oxidation and corrosive loss when subjected to attack by lead containing compounds at temperatures of the order of the operating temperatures of exhaust valves in internal combustion engines; said valve comprising a readily forgeable alloy steel containing a plurality of elements of which the only essential elements necessary to obtain the foregoing characteristics are carbon 0.2% to 1%,

manganese 8% to 12%, chromium 18% to 22%, and aluminum from 1.5% to 3.5%, with the balance substantially all iron; the aluminum content being in excess of the silicon content, if any, in said steel.

4. A readily forgeable alloy steel containing a plurality of elements and characterized by its high resistance to hot oxidation and corrosive loss when subjected to attack by lead containing compounds at temperatures of the order of the operating temperatures of exhaust valves in internal combustion engines; the only essential elements necessary to obtain such characteristics being carbon from 0.2% to 1%, manganese from 8% to 12%, chromium from 18% to 22%, and aluminum from 1.5% to 3.5% with the balance substantially all iron; the silicon content being less than 1% and less than the aluminum content.

5. An internal combustion engine valve comprising the alloy of claim 4.

6. An internal combustion engine valve characterized by its high resistance to hot oxidation and corrosive loss when subjected to attack by lead containing compounds at temperatures of the order of the operating temperatures of exhaust valves in internal combustion engines; said valve comprising an alloy steel containing a plurality of elements of which the only essential elements necessary to obtain the foregoing characteristics are carbon from 0.05% to 3%, manganese from 2% to 20%, chromium from more than 5% to 35% and aluminum from 0.5% to 15%, with the balance substantially all iron; the silicon content being less than 1% and less than the aluminum content.

WALTER R. BREELER.